

## UNITED STATES PATENT OFFICE

2,159,014

## MANUFACTURE OF ARTIFICIAL MATERIALS

Henry Dreyfus, London, England

No Drawing. Application September 18, 1936,  
Serial No. 101,428. In Great Britain September  
23, 1935

4 Claims. (Cl. 8—129)

This invention relates to improvements in the manufacture of yarns and other materials, and is more particularly concerned with processes for the production of yarns and other materials having a basis of cellulose acetate and other organic esters of cellulose, and with the new yarns and other materials produced thereby.

I have found that the resistance to heat of "formed" yarns, foils, films and other materials having a basis of an organic ester of cellulose, i. e., materials formed by shaping and setting compositions containing the organic ester of cellulose, may be increased by esterifying the materials, e. g., with diluted acetic anhydride, in the presence of small proportions of perchloric acid as catalyst. The esterifying agents employed are anhydrides of lower fatty acids, i. e., acids containing not more than six carbon atoms. Suitable anhydrides are propionic, butyric and especially acetic anhydrides. By this means the safe ironing point of yarns and similar materials may be increased so that they may be ironed without damage at higher temperatures than are customary in ironing ordinary cellulose acetate artificial silk. In addition, the treatment reduces the moisture regain of the materials and they acquire a greater resistance to water, and have a substantially greater resistance to the delustering action of hot or boiling aqueous liquids or moist steam. In addition, the affinity of the yarns and other materials for dyestuffs in general is altered. Thus their affinity for the dispersed insoluble dyestuffs now commonly applied to cellulose acetate is materially reduced and a longer time is required to reach any particular depth of colour, and indeed it may not be possible to reach such depth at all. By association, for example, of cellulose acetate yarns or other materials so treated with yarns or other materials of cellulose acetate untreated by the process, differential dyeing effects are therefore obtainable, whilst at the same time the dye has an affinity for the whole of the fabric or other material in which the two types of yarn are associated. Thus, for instance, light and dark blue shades can be produced by the immersion in a dyebath containing an SRA blue dyestuff of a fabric containing ordinary cellulose acetate yarn together with the same yarn which has been subjected to the process of the invention.

An important feature of the new process is that it has the effect of changing the solubility characteristics of the yarns, films and similar materials. Thus for instance by treating a cellulose acetate yarn with acetic anhydride according to

the present invention, a yarn may be produced which is insoluble, or much less soluble in acetone. Similarly, changes in the solubility characteristics occur in the treatment of other yarns used as starting materials in the process of the invention. It is thus possible according to the invention to produce yarns or other materials which it is difficult or even impossible to manufacture by a simple spinning process.

According to the present invention, therefore, materials having improved properties are obtained by acetylation or otherwise esterifying formed filaments, yarns, foils, films and similar materials having a basis of organic esters of cellulose with liquid media comprising anhydrides of lower fatty acids dissolved in diluents with the aid of perchloric acid as catalyst.

It is to be understood that the term "yarn" employed in the present specification, unless otherwise stated, includes yarns in any suitable form, for example in the form of hanks, or on perforated bobbins, or in the form of woven or warp-knitted or other knitted fabrics or similar materials. Bobbins of yarn to be esterified preferably have an open wind.

The invention will hereinafter be described with reference to the acetylation of yarns in hank or similar form, but it is to be understood that it is also applicable to the acetylation of yarns in other forms, e. g., as fabrics and of films, foils and similar materials, and to esterification of yarns, films and similar materials with anhydrides of other lower fatty acids.

The diluent employed, which is a non-solvent for the yarn under treatment, is preferably inert thereto, though it may have a swelling action on the yarn. Good results may be obtained with hydrocarbon diluents, for example benzene, xylene or other homologues of benzene, tetra- and decahydronaphthalenes, and kerosene or other high boiling petroleum hydrocarbons and also ethers, e. g., normal and iso butyl and amyl ethers, carbon tetrachloride and other non-solvent chlorinated hydrocarbons.

When inert diluents are employed they may contain small proportions of swelling agents for the cellulose ester, e. g., acetone, methylene ethylene ether, methylene dichloride and especially acetic acid. For example, the swelling agent may be present in a proportion of 25% or 50% of the weight of the yarn or other material.

The degree of dilution may be adjusted so as to prevent swelling or so as to obtain some swelling of the yarn. In any case, it should be such as to prevent any solution or incipient solution

of the yarn or any fusing together of the filaments, and, further, it may be adjusted to prevent any substantial change in the lustre or quality of the material. A given amount of acetic anhydride may, for example, be dissolved in 7 or 8 or 10 up to 20 times or more its weight of xylene or other hydrocarbon. The higher dilutions are particularly conducive to avoiding change in the lustre and to avoiding shrinkage due to the swelling action of the anhydride. In this connection it may be mentioned that the tendency of stretched yarn to shrink is considerably less than that of normal yarn. The amount of acetic anhydride no the weight of the yarn 15 may vary very considerably according to the degree of acetylation required and the amount of the change in the properties of the material which it is desired to bring about. It is usually sufficient to use an amount of anhydride from half to twice the weight of the material, e. g., a proportion of 1-1½ times its weight.

The reaction is preferably carried out under atmospheric pressure, though it may be effected at subatmospheric pressure or at pressures in excess of atmospheric, for example, pressures of 20 pound per square inch or more.

The materials may be impregnated with the catalyst prior to their introduction into the acetylating medium, but preferably the catalyst is 30 present in the medium. The perchloric acid may be introduced into the acetylating medium as such, or it may be formed therein by reaction between a perchlorate, for example sodium, calcium, magnesium or zinc perchlorate and a suitable 35 acid, for example phosphoric acid. In such case the acid may be present in an amount at least sufficient theoretically to convert the whole of the perchlorate into perchloric acid, or it may be present in smaller proportions so that a mixture 40 of perchlorate and perchloric acid is obtained.

The best proportion of perchloric acid to be employed as catalyst will depend upon various factors, for example upon the duration of acetylation, the degree of acetylation required and the 45 nature of the yarn or other material to be acetylated. In the case of acetylation of ordinary cellulose acetate yarn for periods of about an hour a proportion of about .1-2% of perchloric acid on the weight of the yarn, or the use of a medium containing perchloric acid in a concentration of about .01-.005%, gives very good results. Yarns stretched or stretched and shrunk appear 50 to be rendered by such operation more resistant to the process of acetylation according to the present invention, and it is therefore necessary in general to employ more vigorous conditions, for example a longer period of time or, what is preferred, a somewhat higher proportion of catalyst. For example, in treating stretched yarns 55 the catalyst is preferably employed in a proportion of the order of .5 to 1% on the weight of the yarns, or in a concentration in the acetylating medium of about .05-.025%, the other conditions being as indicated above. The diluent, for example benzene, may be present in proportion of about 20 times the weight of the yarn or other material, and, as indicated above, the presence of a small proportion of acetic acid or 60 other swelling agent, for example a proportion of about 10 to 20 or 50% on the weight of the material, appears to improve the properties of the product obtained. The proportion of acetylating agent will depend upon the degree of acetylation which is required, but, in general, it is

preferably of the order of 150 to 200% on the weight of the material.

The starting material may be a yarn produced by the ordinary spinning process, or it may be a 5 yarn treated by any suitable after-treatment process, for example stretching, shrinking, dyeing or other processes. For example, the yarn subsequent to its manufacture may be subjected to a stretching treatment designed to increase its tenacity, e. g., with the aid of dioxane or other 10 suitable solvent, or in the presence of steam or hot water, as described in United States specification S. Nos. 4,510 and 4,511 filed February 1, 1935. The stretching treatment may, for example, be such as to extend the yarn by 200-500% 15 or even 1000% or more of its original length. Such yarns have an extremely high tenacity which is reflected in the final product treated according to the present invention. Such stretched 20 yarns, or even ordinary artificial silk materials, 25 may, if desired, be subjected to a shrinking treatment to increase their extensibility, for example a shrinking treatment carried out with the aid of latent solvents (see United States Patent No. 2,058,422). As stated above, the stretching of 30 yarns appears to render them more resistant to the process of the present invention, and in general therefore it is necessary to employ more vigorous conditions, e. g., a higher proportion of catalyst, when acetylating such yarns than 35 when normal yarns are acetylated. It is found that the resistance to creasing of stretched yarns 40 may be increased by the process of the present invention.

The reaction between the cellulose ester yarn 35 and the acetylating agent may be carried out in any suitable manner, for example as a batch process. Thus hanks may be immersed for the appropriate period in the acetylation mixture, or the mixture may be pumped or sucked through 40 a perforated bobbin or other package of the yarn.

#### Example

The following example illustrates the production of an improved yarn according to the process of the present invention. 20 parts by weight 45 of ordinary dry spun cellulose acetate yarn are treated for about one hour in a mixture consisting of 400 parts by weight of benzene, about 40 parts by weight of acetic anhydride, 3 parts by weight of acetic acid and .04 part by weight of perchloric acid. After washing and drying a 50 yarn is obtained which is practically insoluble in acetone, has an increased acetyl content, an improved resistance to ironing and to treatment 55 with hot aqueous media and a decreased affinity for the ordinary cellulose acetate dyestuffs.

If, instead of normal yarn, a yarn which has been stretched, for example, to 400 to 600% of its original length, is treated the weight of catalyst should be increased to about .1 to .15 part.

Having now described my invention, what I desire to secure by Letters Patent is:

1. Process for the production of improved artificial materials, which comprises acetylating 65 formed filaments, yarns, foils, films and similar materials having a basis of acetone-soluble cellulose acetate with non-solvent liquid media comprising acetic anhydride dissolved in a suitable diluent with the aid of perchloric acid as 70 catalyst and continuing the acetylation until products having a reduced solubility in acetone are obtained.

2. Process for the production of improved artificial materials, which comprises acetylating nor- 75

- 5 mal acetone-soluble cellulose acetate filaments, yarns and similar materials with a non-solvent liquid medium containing acetic anhydride dissolved in a suitable diluent with the aid of perchloric acid as catalyst in a proportion of the order of 0.1 to 0.2% of the weight of the materials and continuing the acetylation until products having a reduced solubility in acetone are obtained.
- 10 13. Process for the production of improved artificial materials, which comprises acetylating stretched acetone-soluble cellulose acetate filaments, yarns and similar materials with a non-solvent liquid medium comprising acetic anhydride dissolved in a suitable diluent with the aid of perchloric acid as catalyst in a proportion of the order of 0.5 to 1% of the weight of the materials and continuing the acetylation until products having a reduced solubility in acetone are obtained. 15
- 15 HENRY DREYFUS.